



US006015593A

# United States Patent [19]

Yonkoski et al.

[11] Patent Number: 6,015,593

[45] Date of Patent: \*Jan. 18, 2000

- [54] **METHOD FOR DRYING A COATING ON A SUBSTRATE AND REDUCING MOTTLE**

[75] Inventors: **Roger K. Yonkoski**, Woodbury, Minn.; **Brian L. Strobush**, Kingwood, Tex.; **Thomas J. Ludemann**, Maplewood; **Robert A. Yapel**, Oakdale, both of Minn.

[73] Assignee: **3M Innovative Properties Company**, St. Paul, Minn.

[\*] Notice: This patent issued on a continued prosecution application filed under 37 CFR 1.53(d), and is subject to the twenty year patent term provisions of 35 U.S.C. 154(a)(2).

[21] Appl. No.: **08/624,164**

[22] Filed: **Mar. 29, 1996**

[51] Int. Cl.<sup>7</sup> ..... **B05D 3/02**

[52] U.S. Cl. ..... **427/379; 427/402**

[58] Field of Search ..... **427/372.2, 379, 427/385.5, 402**

4,847,175 7/1989 Pavlisko et al. .... 430/58  
 4,872,270 10/1989 Fronheiser et al. ....  
 4,894,927 1/1990 Ogawa et al. ....  
 4,999,927 3/1991 Durst et al. ....  
 5,001,845 3/1991 Norz et al. ....  
 5,010,659 4/1991 Treleven ....  
 5,060,396 10/1991 Hansen ....  
 5,077,912 1/1992 Ogawa et al. .... 427/379  
 5,136,790 8/1992 Hagen et al. ....  
 5,147,690 9/1992 Faust et al. ....  
 5,298,292 3/1994 Dilko et al. .... 427/372.2  
 5,394,622 3/1995 Evans et al. ....  
 5,433,973 7/1995 Wallack et al. ....  
 5,468,603 11/1995 Kub .... 430/617  
 5,532,121 7/1996 Yonkoski et al. .... 430/617

**FOREIGN PATENT DOCUMENTS**

|            |         |            |
|------------|---------|------------|
| 236 186 A1 | 5/1986  | Germany .  |
| 620766     | 7/1978  | U.S.S.R. . |
| 1276889    | 12/1986 | U.S.S.R. . |

*Primary Examiner—Shrive Beck  
 Assistant Examiner—Bret Chen  
 Attorney, Agent, or Firm—Charles D. Levine*

[57] **ABSTRACT**

An apparatus and method for evaporating a coating solvent

[56] **References Cited**

## U.S. PATENT DOCUMENTS

- |           |         |                          |
|-----------|---------|--------------------------|
| 3,494,048 | 2/1970  | Du Fresne .              |
| 3,849,904 | 11/1974 | Villalobos .             |
| 4,051,278 | 9/1977  | Democh ..... 427/326     |
| 4,365,423 | 12/1982 | Arter et al. ..... 34/23 |
| 4,569,658 | 2/1986  | Wiggins et al. .         |
| 4,594,266 | 6/1986  | Lemaire et al. .         |
| 4,634,840 | 1/1987  | Yamagishi et al. .       |
| 4,698,914 | 10/1987 | Shu et al. .             |
| 4,843,731 | 7/1989  | Vits .                   |

- |           |         |                      |           |
|-----------|---------|----------------------|-----------|
| 4,847,175 | 7/1989  | Pavlisko et al. .... | 430/58    |
| 4,872,270 | 10/1989 | Fronheiser et al. .  |           |
| 4,894,927 | 1/1990  | Ogawa et al. .       |           |
| 4,999,927 | 3/1991  | Durst et al. .       |           |
| 5,001,845 | 3/1991  | Norz et al. .        |           |
| 5,010,659 | 4/1991  | Treleven. .          |           |
| 5,060,396 | 10/1991 | Hansen .             |           |
| 5,077,912 | 1/1992  | Ogawa et al. ....    | 427/379   |
| 5,136,790 | 8/1992  | Hagen et al. .       |           |
| 5,147,690 | 9/1992  | Faust et al. .       |           |
| 5,298,292 | 3/1994  | Dilko et al. ....    | 427/372.2 |
| 5,394,622 | 3/1995  | Evans et al. .       |           |
| 5,433,973 | 7/1995  | Wallack et al. .     |           |
| 5,468,603 | 11/1995 | Kub .....            | 430/617   |
| 5,532,121 | 7/1996  | Yonkoski et al. .... | 430/617   |

## FOREIGN PATENT DOCUMENTS

- 236 186 A1 5/1986 Germany .  
 620766 7/1978 U.S.S.R. .  
 1276889 12/1986 U.S.S.R. .

*Primary Examiner*—Shrive Beck

*Assistant Examiner*—Bret Chen

*Attorney, Agent, or Firm*—Charles D. Levine

[57] ABSTRACT

An apparatus and method for evaporating a coating solvent from a coating on a substrate and for minimizing the formation of mottle. The coating is heated with a first drying gas at no higher than a first heat transfer rate. The first heat transfer rate is created by a first heat transfer coefficient and a first temperature difference between the first coating temperature and the first drying gas temperature. The first heat transfer rate causes maximum evaporation of the coating solvent yet insignificant formation of mottle when the coating is at the first coating thickness and the first coating viscosity.

**40 Claims, 13 Drawing Sheets**









**Fig. 3**  
PRIORITY ART



**Fig. 4**  
PRIORITY ART



Fig. 6

**Fig. 7****Fig. 8****Fig. 9**



Fig. 10



**Fig. 11**



**Fig. 12**

**Fig. 13****Fig. 14**



Fig. 15



Fig. 16

**Fig. 17****Fig. 18**



Fig. 19



Fig. 20

**Fig. 21****Fig. 22**



Fig. 23

## METHOD FOR DRYING A COATING ON A SUBSTRATE AND REDUCING MOTTLE

### FIELD OF THE INVENTION

The present invention relates to methods for drying coatings on a substrate and more particularly to methods for drying coatings used in making imaging articles.

### BACKGROUND OF THE INVENTION

The production of high quality articles, particularly photographic, photothermographic, and thermographic articles, consists of applying a thin film of coating solution onto a continuously moving substrate. Thin films can be applied using a variety of techniques including: dip coating, forward or reverse roll coating, wire-wound coating, blade coating, slot coating, slide coating, and curtain coating (see for example L. E. Scriven; W. J. Suszynski; *Chem. Eng. Prog.* 1990, September, p. 24). Coatings can be applied as single layers or as two or more superposed layers. While it is usually most convenient for the substrate to be in the form of a continuous substrate, it can also be in the form of a succession of discrete sheets.

The initial coating is either a mixture of solvent and solids or a solution and must be dried to obtain the final dried article. While the cost of a coating process is determined by the coating technique, the cost of a drying process is often proportional to the desired line speed (see E. D. Cohen; E. J. Lightfoot; E. B. Gutoff; *Chem. Eng. Prog.* 1990, September, p. 30). The line speed is limited by the capabilities of the oven. To reduce costs, it is desirable that the removal of solvent from the coating be as efficient as possible. This is generally accomplished by transferring heat to the coated article as efficiently as possible. This is often accomplished by increasing the velocity of the drying gas at the coating surface, thereby increasing heat transfer and solvent evaporation and thus drying the coating more quickly. The resulting turbulent air, however, increases the tendency for defect formation.

The process of applying a coating to and drying that coating on a substrate can inherently create defects, including Benard cells, orange peel, and mottle. Benard cells are defects arising from circulatory motion within the coating after it has been applied (see C. M. Hanson; P. E. Pierce; *Cellular Convection in Polymer Coatings-An Assessment*, 12 Ind. Eng. Chem. Prod. Res. Develop. 1973, p. 67).

Orange peel is related to Benard cells. Orange peel is most common in fluid coatings which have a high viscosity to solids ratio. This is due to the tendency of such systems to "freeze in" the topography associated with Benard cells upon loss of relatively small amounts of solvent. The topography can be observed as a small scale pattern of fine spots like the surface of an orange peel. The scale of the pattern is on the order of millimeters and smaller.

Mottle is an irregular pattern or non-uniform density defect that appears blotchy when viewed. This blotchiness can be gross or subtle. The pattern may even take on an orientation in one direction. The scale can be quite small or quite large and may be on the order of centimeters. Blotches may appear to be different colors or shades of color. In black-and-white imaging materials, blotches are generally shades of gray and may not be apparent in unprocessed articles but become apparent upon development. Mottle is usually caused by air movement over the coating before it enters the dryer, as it enters the dryer, or in the dryer (see for example, "Modern Coating and Drying Technology," Eds. E. D. Cohen, E. B. Gutoff, VCH Publishers, N.Y., 1992; p. 288).

Mottle is a problem that is encountered under a wide variety of conditions. For example, mottle is frequently encountered when coatings comprising solutions of a polymeric resin in an organic solvent are coated onto webs or sheets of synthetic organic polymer substrates. Mottle is an especially severe problem when the coating solution contains a volatile organic solvent but can also occur to a significant extent even with aqueous coating compositions or with coating compositions using an organic solvent of low volatility. Mottle is an undesirable defect because it detracts from the appearance of the finished product. In some instances, such as in imaging articles, it is further undesirable because it adversely affects the functioning of the coated article.

Substrates that have been coated are often dried using a drying oven which contains a drying gas. The drying gas, usually air, is heated to a suitable elevated temperature and brought into contact with the coating in order to bring about evaporation of the solvent. The drying gas can be introduced into the drying oven in a variety of ways. Typically, the drying gas is directed in a manner which distributes it uniformly over the surface of the coating under carefully controlled conditions that are designed to result in a minimum amount of disturbance of the coated layer. The spent drying gas, that is, drying gas which has become laden with solvent vapor evaporated from the coating, is continuously discharged from the dryer. Many industrial dryers use a number of individually isolated zones to allow for flexibility in drying characteristics along the drying path. For example, U.S. Pat. No. 5,060,396 describes a zoned cylindrical dryer for removing solvents from a traveling substrate. The multiple drying zones are physically separated, and each drying zone may operate at a different temperature and pressure. Multiple drying zones are desirable because they permit the use of successively lower solvent vapor composition. German Pat. No. DD 236,186 describes the control of humidity and temperature of each drying zone to effect maximum drying at minimum cost. Soviet Pat. No. SU 620766 describes a multistage timber dryer with staged temperature increases that reduce the stress within the timber.

Usually, when multiple zones are present in an oven, they are isolated from one another. The coated substrate is transferred between the zones through a slot. In order to minimize the air and heat flow between zones and to be able to effectively control the drying conditions in each zone, this slot typically has as small a cross-section as possible that will still allow the substrate to pass between zones. However, the adjacent zones are in communication with one another through the slot and thus there is typically a pressure difference between zones. Air flows from one zone to another; and since the dimensions of the slot are small, the air gas velocity is high. Therefore the slots between ovens tend to be sources for mottle defects.

U.S. Pat. No. 4,365,423 discloses an apparatus and method for drying to reduce mottle. FIG. 1 shows an embodiment of this invention. The drying apparatus 2A uses a foraminous shield 4A to protect the liquid coating 6A from air disturbances. The foraminous shield 4A is described to be a screen or perforated plate that sets up a "quiescent" zone above the substrate promoting uniform heat and mass transfer conditions. The shield 4A is also noted to restrict the extent to which spent drying gas, which is impinged toward the liquid coating 6A, comes in contact with the surface of the coating. This method is reported to be especially advantageous in drying photographic materials, particularly those comprising one or more layers formed from coating compositions that contain volatile organic solvents. This apparatus and method has the limitation that it slows the rate of drying.

U.S. Pat. No. 4,999,927 discloses another apparatus and method for drying a liquid layer that has been applied to a carrier material moving through a drying zone and which contains both vaporizable solvent components and non-vaporizable components. FIG. 2 illustrates this apparatus 2B and method. Drying gas flows in the direction of the carrier material 8B and is accelerated within the drying zone in the direction of flow. In this manner, laminar flow of the boundary layer of the drying gas adjacent to the liquid layer on the carrier material is maintained. By avoiding turbulent air flow, mottle is reduced.

Examples of two other known drying apparatuses and methods are shown in FIG. 3 and 4. FIG. 3 schematically shows a known drying apparatus 2C in which air flows (see arrows) from one end of an enclosure to the other end. The airflow is shown in FIG. 3 as being parallel and counter to the direction of travel of the coated substrate (i.e., counter-current). Parallel cocurrent airflow is also known.

FIG. 4 schematically shows a known drying apparatus 2D which involves the creation of impingement airflow (see arrows), that is more perpendicular to the plane of the substrate 8D. The impinging air also acts as a means for floating or supporting the substrate through the oven.

U.S. Pat. No. 4,051,278 describes a method for reducing mottle caused by solvent evaporation in the coating zone. Coating a substrate with reduced mottle, such as coating a composition comprising a film-forming material in an evaporable liquid vehicle onto a flexible web or synthetic organic polymer, is achieved by maintaining at least two of the following at a temperature substantially equivalent to the equilibrium surface temperature of the coated layer at the coating zone: (1) the temperature of the atmosphere at the location of coating; (2) the temperature of the coating composition at the location of coating; and (3) the temperature of the substrate at the coating zone. The equilibrium surface temperature is defined as the temperature assumed by the surface of a layer of the coating composition under steady state conditions of heat transfer following evaporative cooling of the layer at the coating zone. After coating, drying of the coated layer is carried out by conventional techniques. This invention includes methods of drying while preventing mottle formation by controlling temperature (i.e., by cooling) at the coating zone and does not address temperature control or mottle formation within the drying oven. Furthermore, this method would be useful only for coatings that cool significantly due to evaporative cooling which subsequently causes mottle.

U.S. Pat. No. 4,872,270 describes a method of drying latex paint containing water and one or more high boiling organic solvents coated onto a carrier film. The process yields a dried paint layer free of blisters and bubble defects. The coated film is passed continuously through a series of at least three drying stages in contact with warm, moderately humid air and more than half of the heat required for evaporation is supplied to the underside of the film. Drying conditions in at least each of the first three stages are controlled to maintain a film temperature profile which causes the water to evaporate at a moderate rate but more rapidly than the organic solvents, thus achieving coalescence of the paint and avoiding the trapping of liquids in a surface-hardened paint layer. Bubble formation is reportedly eliminated by controlling the vapor pressure of the volatile solvent within the film. The formation of mottle occurs due to a different mechanism than blisters and requires different methods for control and elimination.

U.S. Pat. No. 4,894,927 describes a process for drying a moving web coated with a coating composition containing a

flammable organic solvent. The web is passed through a closed-type oven filled with an inert gas and planer heaters on top and bottom of the web. The coating surface is reported to be barely affected by movement of the inert drying gases due to the small amounts of gas required. No discussion of the criticality of the gas flow system or of the need to prevent mottle is given.

U.S. Pat. No. 5,077,912 describes a process for drying a continuously traveling web coated with a coating composition containing an organic solvent. The coating is first dried using hot air until the coating is set-to-touch. It is sufficient that the drying conditions, such as temperature and hot air velocity, are adjusted so as to obtain the set-to-touch condition. Set-to-touch corresponds to a viscosity of  $10^8$  to  $10^{10}$  15 poise. Residual solvent is then removed using a heated roll. This method is said to reduce drying defects, decrease drying time, and reduce oven size. No discussion on the construction of the oven, methods of drying, or the criticality of the gas flow system and path is given.

U.S. Pat. No. 5,147,690 describes a process and apparatus for drying a liquid film on a substrate which includes a lower gas or air supply system and an upper gas or air supply system. Heated gas on the underside of the substrate forms a carrying cushion for the substrate and at the same time 25 supplies drying energy to the substrate. The exhaust air is carried away through return channels. Slots for the gas supply and return are arranged alternately in the lower gas system. The upper gas or air supply system has a greater width than the lower gas or air supply system. In the upper 30 gas or air supply system, the supply air or gas is diverted by baffles onto the substrate and returned over the substrate web as return air or gas. The upper gas or air supply system is subdivided into sections for the supply air and exhaust air, each section includes two filter plates of porous material.

U. S. Pat. No. 5,433,973 discloses a method of coating a magnetic recording media onto a substrate, wherein the coating is substantially free of Benard cells. The method comprises the steps of: (a) providing a dispersion comprising a polymeric binder, a pigment, and a solvent; (b) coating the dispersion onto the surface of a substrate; (c) drying the dispersion; (d) calculating values comprising  $\mu$ ,  $\beta$ , and  $d$  40 representing the viscosity, temperature gradient, and wet caliper of the dispersion respectively; and (e) during the course of carrying out steps (a), (b), and (c), maintaining the ratio

$$\frac{\beta d^2}{\mu}$$

50 below a threshold value sufficient to substantially prevent the formation of Benard Cells in the magnetic recording media coating. No discussion of the interior of the drying oven and arrangement of air inlets and exhausts is given.

55 A number of methods involve the control of the drying gas within the oven. For example, U.S. Pat. No. 5,001,845 describes a control system for an industrial dryer used to remove a flammable solvent or vapors from a traveling web of material. Sensors within each zone measure the oxygen 60 content of the pressurized atmosphere. If the oxygen content exceeds a given limit, an inert gas is added. At the same time, the pressure is maintained within the oven body by releasing excess gas to the atmosphere.

U.S. Pat. No. 5,136,790 describes a method and apparatus 65 for drying a continuously moving web carrying a liquid, wherein the web is passed through a dryer in which the web is exposed to a recirculating flow of heated drying gas.

Exhaust gas is diverted and discharged from the recirculating gas flow at a gas velocity which is variable between maximum and minimum levels, and makeup gas is added to the recirculating gas flow at a gas velocity which is also variable between maximum and minimum levels. A process variable is sensed and compared to a selected set point. A first of the aforesaid flow rates is adjusted to maintain the process variable at the selected set point, and a second of the aforesaid flow rates is adjusted in response to adjustments to the first drying gas velocity in order to insure that the first drying gas velocity remains between its maximum and minimum levels. No discussion of the interior of the drying oven and arrangement of air inlets and exhausts is given.

Soviet Pat. No. SU 1,276,889 describes a method for controlling drying gas by controlling the air gas velocity within the oven. In this method, fan speed in one zone is adjusted, controlling the air flow rate, in order to maintain the web temperature at the outlet to a specified temperature. This approach is limited in that increasing the air gas velocity in order to meet a drying specification can lead to mottle.

The physical state of the drying web can also be used to control the drying ovens. For example, in Soviet Pat. No. SU 1,276,889, noted above, the temperature of the web at the outlet of the oven was used to set the air flow rate.

U.S. Pat. No. 5,010,659 describes an infrared drying system for monitoring the temperature, moisture content, or other physical property at particular zone positions along the width of a traveling web, and utilizing a computer control system to energize and control for finite time periods a plurality of infrared lamps for equalizing physical property and drying the web. The infrared drying system is particularly useful in the graphic arts industry, the coating industry and the paper industry, as well as any other applications requiring physical property profiling and drying of the width of a traveling web of material. No discussion of the interior of the drying oven and arrangement of air inlets and exhausts is given.

U.S. Pat. No. 4,634,840 describes a method for controlling the drying temperature in an oven used for heat-treating thermoplastic sheets and films. A broad and continuous sheet or film is uniformly heated in a highly precise manner and with a specific heat profile by using a plurality of radiation heating furnaces, wherein in the interior of each radiation heating furnace, a plurality of rows of heaters are arranged rectangularly to the direction of delivery of the sheet or film to be heated. A thermometer for measuring the temperature of the sheet or film is arranged in the vicinity of an outlet for the sheet or film outside each radiation heating furnace. Outputs of heaters arranged within the radiation heating furnaces located just before the respective thermometers are controlled based on the temperatures detected by the respective thermometers by using a computer.

Two other patents address drying problems, but fail to address the problem of mottle. U.S. Pat. No. 3,849,904 describes the use of a mechanical restriction of air flow at the edge of a web. Adjustable edge deckles are noted as forming a seal with the underside of a fabric allowing for different heating conditions to occur at the edge. This allows the edge of the fabric to be cooled while the remainder of the fabric is heated. This approach, however, is not advantageous when a polymer substrate is used. Possible scratching of the polymer substrate can generate small particulates which can be deposited on the coating. U.S. Pat. No. 3,494,048 describes the use of mechanical means to divert air flow at the edge of the web. Baffles are noted as deflecting air and preventing air from penetrating behind paper in an ink dryer

and from lifting the paper from a drum. Keeping the paper on the drum prevents the drying ink from being smeared.

A need exists for a drying apparatus and method which reduces, if not eliminates, one or more coating defects such as mottle and orange peel, yet permits high throughput. In addition to the drying of coatings used to make photothermographic, thermographic, and photographic articles, the need for improved drying apparatus and methods extends to the drying of coatings of adhesive solutions, magnetic recording solutions, priming solutions, and the like.

#### SUMMARY OF THE INVENTION

The present invention can be used to dry coated substrates, and particularly to dry coated substrates used in the manufacture of photothermographic, thermographic, and photographic articles. More importantly, the present invention can do this without introducing significant mottle and while running at higher web speeds than known drying methods.

One embodiment includes a method for evaporating a coating solvent from a coating on a substrate and minimizing the formation of mottle as the coating solvent is evaporating. The substrate has a first substrate surface and a second substrate surface. The method includes a step of applying the coating onto the first substrate surface of the substrate at a first coating thickness, the coating having a first coating viscosity and a first coating temperature when applied to the first substrate surface. Another step includes heating the coating with a first drying gas at no higher than a first heat transfer rate, the first drying gas having a first drying gas temperature, the first heat transfer rate being created by a first heat transfer coefficient and a first temperature difference between the first coating temperature and the first drying gas temperature. The first heat transfer rate causes maximum evaporation of the coating solvent yet insignificant formation of mottle when the coating is at the first coating thickness and the first coating viscosity. The coating is heated predominantly by the first drying gas adjacent to the substrate second surface. Another step includes heating the coating with a second drying gas at no higher than a second heat transfer rate after a first portion of the coating solvent has evaporated and the coating has a second wet thickness and a second viscosity. The coating has a second coating temperature just before being heated by the second drying gas. The second wet thickness is less than the first wet thickness. The second drying gas has a second drying gas temperature. The second heat transfer rate is created by a second heat transfer coefficient and a second temperature difference between the second coating temperature and the second drying gas temperature. The second heat transfer rate causing a maximum evaporation yet insignificant formation of mottle when the coating is at the second wet thickness and the second viscosity. At least one of the second heat transfer coefficient and the second drying gas temperature is greater than the respective first heat transfer coefficient and first drying gas temperature. The coating is heated predominantly by the drying gas adjacent to the substrate second surface.

Another embodiment includes a method for evaporating a coating solvent from a coating on a first substrate surface and minimizing the formation of mottle in the coating as the coating solvent is evaporating. The coating has a first coating temperature  $T_{c1}$  when applied to the substrate. The substrate also has a second substrate surface opposite to the first substrate surface. The method includes a step of providing a first evaporating environment for the coating. The

first evaporating environment contains a drying gas which heats the coating predominantly by flowing adjacent to the second substrate surface. Another step includes flowing the drying gas adjacent to the second substrate surface at a first drying gas velocity to create a first heat transfer coefficient  $h_1$  and heating the drying gas to a first drying gas temperature  $T_{gas1}$  such that the product

$$h_1 (T_{gas1} - T_{c1})$$

is not greater than a first threshold value such that the formation of mottle is substantially prevented. Another step includes determining the first threshold value for the product

$$h_1 (T_{gas1} - T_{c1}).$$

Another step includes transporting the substrate through the first evaporating environment.

Another embodiment includes an apparatus for evaporating a coating solvent from a coating on a substrate and minimizing the formation of mottle as the coating solvent is evaporating. The substrate has a first substrate surface and a second substrate surface. The apparatus includes means for applying the coating onto the first substrate surface of the substrate at a first coating thickness. The coating has a first coating viscosity and a first coating temperature when applied to the first substrate surface. The apparatus further includes means for heating the coating with a first drying gas at no higher than a first heat transfer rate. The first drying gas has a first drying gas temperature. The first heat transfer rate is created by a first heat transfer coefficient and a first temperature difference between the first coating temperature and the first drying gas temperature. The first heat transfer rate causes maximum evaporation of the coating solvent yet insignificant formation of mottle when the coating is at the first coating thickness and the first coating viscosity. The coating is heated predominantly by the first drying gas adjacent to the substrate second surface. The apparatus further includes means for heating the coating with a second drying gas at no higher than a second heat transfer rate after a first portion of the coating solvent has evaporated and the coating has a second wet thickness and a second viscosity. The coating has a second coating temperature just before being heated by the second drying gas. The second wet thickness is less than the first wet thickness. The second drying gas has a second drying gas temperature. The second heat transfer rate is created by a second heat transfer coefficient and a second temperature difference between the second coating temperature and the second drying gas temperature. The second heat transfer rate causes a maximum evaporation yet insignificant formation of mottle when the coating is at the second wet thickness and the second viscosity, at least one of the second heat transfer coefficient and the second drying gas temperature being greater than the respective first heat transfer coefficient and first drying gas temperature. The coating is heated predominantly by the drying gas adjacent to the substrate second surface.

Another embodiment includes an apparatus for evaporating a coating solvent from a coating on a first substrate surface and minimizing the formation of mottle in the coating as the coating solvent is evaporating. The coating has a first coating temperature  $T_{c1}$  when applied to the substrate. The substrate also has a second substrate surface opposite to the first substrate surface. The apparatus includes means for providing a first evaporating environment for the coating. The first evaporating environment contains a drying gas which heats the coating predominantly by flowing adjacent to the second substrate surface. Means for flowing the drying gas adjacent to the second substrate surface at a first drying gas velocity creates a first heat transfer coefficient  $h_1$  and heats the drying gas to a first drying gas temperature  $T_{gas1}$  such that the product

$h_1 (T_{gas1} - T_{c1})$  is not greater than a first threshold value such that the formation of mottle is substantially prevented. The apparatus further includes means for determining the first threshold value for the product

$$h_1 (T_{gas1} - T_{c1}).$$

The apparatus further includes means for transporting the substrate through the first evaporating environment.

As used herein:

"photothermographic article" means a construction comprising at least one photothermographic emulsion layer and any substrates, top-coat layers, image receiving layers, blocking layers, antihalation layers, subbing or priming layers, etc.

"thermographic article" means a construction comprising at least one thermographic emulsion layer and any substrates, top-coat layers, image receiving layers, blocking layers, antihalation layers, subbing or priming layers, etc.

"emulsion layer" means a layer of a photothermographic element that contains the photosensitive silver halide and non-photosensitive reducible silver source material; or a layer of the thermographic element that contains the non-photosensitive reducible silver source material.

Other aspects, advantages, and benefits of the present invention are disclosed and apparent from the detailed description, examples, and claims.

#### BRIEF DESCRIPTION OF THE DRAWINGS

The foregoing advantages, construction, and operation of the present invention will become more readily apparent from the following description and accompanying drawings.

FIG. 1 is a side view of a known drying apparatus;

FIG. 2 is a side view of another known drying apparatus;

FIG. 3 is a side schematic view of another known drying apparatus,

FIG. 4 is a side schematic view of another known drying apparatus;

FIG. 5 is a side view of a drying apparatus in accordance with the present invention;

FIG. 6 is a partial side view of the drying apparatus shown in FIG. 5;

FIG. 7 is a partial sectional view of the drying apparatus shown in FIG. 6;

FIG. 8 is a partial sectional view of the drying apparatus shown in FIG. 6;

FIG. 9 is a sectional front view of the drying apparatus shown in FIG. 6;

FIG. 10 is a side schematic view of an air foil and an air bar which are shown in FIGS. 5-9;

FIG. 11 is a side view of an alternative embodiment of the drying apparatus shown in FIGS. 5-10;

FIG. 12 is a side view of alternative embodiment of the drying apparatus shown in FIGS. 5-11;

FIG. 13 is a graph illustrating the constant temperature of a drying gas within a drying oven and the resulting coating temperatures as a function of distance traveled within the oven;

FIG. 14 is a graph illustrating the maximum allowable heat transfer rate and actual heat transfer rate to the coating as a result of the constant drying gas temperature illustrated in FIG. 13;

FIG. 15 is a graph illustrating the resulting coating temperatures as a function of distance traveled within an oven when the coating is subjected to two different drying gas temperatures;

FIG. 16 is a graph illustrating the maximum allowable heat transfer rate and the actual heat transfer rate to the coating as a result of being subjected to the two drying gas temperatures illustrated in FIG. 15;

FIG. 17 is a graph illustrating the resulting coating temperatures as a function of distance traveled within an oven when the coating is subjected to three different drying gas temperatures;

FIG. 18 is a graph illustrating the maximum allowable heat transfer rate and the actual heat transfer rate to the coating as a result of being subjected to the three drying gas temperatures illustrated in FIG. 17;

FIG. 19 is a graph illustrating the resulting coating temperatures as a function of distance within an oven when the coating is subjected to fifteen different drying gas temperatures;

FIG. 20 is a graph illustrating the maximum allowable heat transfer rate and the actual heat transfer rate to the coating as a result of being subjected to the fifteen drying gas temperatures illustrated in FIG. 19;

FIG. 21 is a graph illustrating the resulting coating temperatures as a function of distance within an oven when the coating is subjected to fifteen different drying gas temperatures where the maximum allowable heat transfer rate increases along the length of the oven;

FIG. 22 is a graph illustrating the maximum allowable heat transfer rate and the actual heat transfer rates to the coating as a result of being subjected to the fifteen drying gas temperatures illustrated in FIG. 19; and

FIG. 23 is a side view of another embodiment of the drying apparatus shown generally in FIG. 5.

#### DETAILED DESCRIPTION OF THE INVENTION

A drying apparatus 10 is illustrated generally in FIG. 5 and more specifically in FIGS. 6-10. This drying apparatus 10 is useful for drying a coating 12 which has been applied to (i.e., coated onto) a substrate 14 forming a coated substrate 16. When the coating 12 comprises a film-forming material or other solid material dissolved, dispersed, or emulsified in an evaporable liquid vehicle, drying means evaporating the evaporable liquid vehicle (e.g., solvent) so that a dried, film or solids layer (e.g., an adhesive layer or a photothermographic layer) remains on the substrate 14. Hereinafter, the more generic "evaporable liquid vehicle" will herein be referred to as a "solvent."

While suitable for a wide variety of coatings, the drying apparatus 10 is particularly suited for drying photothermographic and thermographic coatings to prepare photothermographic and thermographic articles. The drying apparatus 10 has the ability to dry such coatings in a relatively short period of time while minimizing the creation of drying-induced defects, such as mottle. The following disclosure describes embodiments of the drying apparatus 10, embodiments of methods for using the drying apparatus 10, and details pertaining to materials particularly suited for drying by the drying apparatus 10.

#### The Drying Apparatus 10

FIGS. 5-10 show an embodiment of the drying apparatus 10 which generally can include a drying enclosure 17 with a first zone 18 and a second zone 20. The first and second

zones 18, 20 can be divided by a zone wall 22. As will become more apparent later within this disclosure, the first zone 18 is of primary importance. The first zone 18 and the second zone 20 can each provide different drying environment. In addition, the first zone 18 can provide a plurality of drying environments therein, which will be discussed further.

The substrate 14 can be unwound by a substrate unwinder 24, and the coating 12 is shown as being coated onto the substrate 14 by coating apparatus 26. The coated substrate 16 can enter the drying apparatus 10 through a coated substrate entrance 27 and be dried when traveling through the first and second zones 18, 20. The coated substrate can exit the drying apparatus 10 through a coated substrate exit 28 then be wound at the coated substrate winder 29. Although the coated substrate 16 is shown as following an arched path through the first zone 18, the path could be flat or have another shape. And, although the coated substrate 16 is shown being redirected within zone 2 such that the coated web takes three passes through zone 2, the drying apparatus 10 could be designed such that fewer or more passes occur.

The first zone 18 is more specifically shown in FIGS. 6-10 as including a number of air foils 30 which are located below the coated substrate 16 along the length of the first zone 18. The air foils 30 supply drying gas (e.g., heated air, inert gas) toward the bottom surface of the coated substrate 16 such that the coated substrate can ride on a cushion of drying gas. Drying gas is supplied to a group of air foils 30 by an air foil plenum 31.

The temperature and gas velocity of the drying gas supplied from a group of air foils 30 can be controlled by controlling the temperature and pressure of the drying gas in the corresponding air foil plenum 31. Consequently, independent control of the temperature and pressure of the drying gas within each air foil plenum 31 allows for independent control of the temperature and gas velocity of the drying gas supplied by each group of air foils 30.

Although each air foil plenum 31 is shown as supplying a group of either twelve or fifteen air foils 30, other ducting arrangements could be used. An extreme example would be for one air foil plenum 31 to supply drying gas to only one air foil 30. With this arrangement, independent control of the temperature and pressure for each air foil plenum 31 would result in independent control of the temperature and gas velocity of the drying gas exiting from each air foil 30.

Each of the air foils can have a foil slot (the side view of which is shown in FIG. 10) through which a stream of drying gas enters into the drying apparatus 10. The foil slot can have a slot width which is not significantly wider than the substrate width such that mottle on the first and second coating edges is minimized. Setting the width in this way affects the flow of the drying gas around the edges of the substrate. When the foil slot width is approximately equal to or narrower than the width of the substrate, mottle on the edges of the liquid is reduced.

FIG. 10 illustrates the flow of air out of a foil slot of an air foil 30 and FIG. 7 illustrates the length of air foils 30. Because the slot can be made to extend to the ends of the air foil 30, the slot length can virtually be as long as the length of the air foil 30. Because the drying apparatus 10 can be used to dry coated substrates 16 having a widths which are significantly less than the foil slot length (as well coated substrates 16 having widths approximately equal to or even wider than the foil slot length), one or both of the ends of the foil slot can be deckled such that the foil slot length is approximately equal to the width of the narrower coated substrates. The length of the slots can be deckled or adjusted

## 11

by covering more or less of the ends of the slots with a material such as an adhesive tape. Alternatively, a metal plate at each edge of the foil slots could be inwardly and outwardly movable to close off more or less of the foil slot. Also, ends of the slots could be plugged with a material, such as a conformable material (e.g., rubber).

Lower exhaust ports **32** are positioned below the air foils **30** to remove the drying gas, or at least a portion of the drying gas, supplied by the air foils **30**. The drying gas exhausted by a group of lower exhaust ports **32** is exhausted into a lower exhaust plenum **33**. Five lower exhaust plenums **33** are shown, each of which is connected to two lower exhaust ports **32**. Lower exhaust ports **32** are distributed throughout the lower interior portion of the drying apparatus **10** to remove drying gas throughout the drying apparatus **10** rather than at concentrated points. Other similar ducting arrangements are envisioned.

The velocity of the drying gas through a lower exhaust port **32** can largely be controlled by controlling the static pressure difference between the lower interior portion of the drying apparatus **10** (the interior portion below the coated substrate level) and some suitable reference point (e.g., the coating room in which the coating apparatus **26** is positioned; or, each lower exhaust plenum **33**). As a result, independent control of the static pressure difference between the lower interior portion of the drying apparatus **10** and each lower exhaust plenum **33** allows for independent control of the gas velocity exhausted by the group of lower exhaust ports **32** of each lower exhaust plenums **33**.

The combination of the ability to independently control the drying gas supplied by each air foil plenum **31** (temperature and gas velocity) and the ability to independently control the drying gas exhausted by each exhaust plenum **33** allows for the creation of lower subzones within the first zone **18** of the drying apparatus **10**. As shown, the first zone **18** has five lower subzones due to the independent control of five air foil plenums **31** and five lower exhaust plenums **33**. As a result, the five lower subzones can contain drying gas with a unique temperature and a unique gas velocity (or other heat transfer coefficient factor). In other words, the coated substrate **16** can be subjected to five different drying environments (subzones).

The flow direction of the drying gas from the air foils **30** can be controlled based on the configuration of the air foils. As shown in FIG. 10, the air foils **30** can be configured to initially supply drying gas cocurrently with the travel direction of the coated substrate and against the bottom surface of the coated substrate **16** to create a cushion of air on which the coated substrate floats. The airfoils **30** can be designed such that the drying gas flows essentially parallel to the coated substrate **16** and such that the coated substrate **16** floats approximately 0.3 to 0.7 centimeters above the upper portion of the airfoils **30**. While shown as causing cocurrent gas flow to the substrate travel direction, the air foils **30** could be configured to cause the drying gas to impinge on the substrate second surface, to flow generally countercurrently to the substrate travel direction, to flow generally orthogonally to the substrate travel direction, or to flow generally diagonally to the substrate travel direction.

Air bars **34** are located above the coated substrate **16** along the length of the first zone **18**. The air bars **34** can be used to supply top-side gas (e.g., fresh air, inert gas) which can be useful for added drying, to carry away evaporated solvent, and/or to dilute the solvent if it is necessary to control the solvent level within the drying enclosure **17**. The top-side gas is supplied to a group of air bars **34** by an air bar plenum **35**. Although each air bar plenum **35** is shown

## 12

as supplying a particular number of air bars **34**, other ducting arrangements are envisioned. If desired, the drying apparatus **10** can be used such that no gas is supplied by the air bars **34** when top-side gas is not needed or desired (e.g., when the drying apparatus **10** is filled with inert gas).

The velocity of the top-side gas supplied from a group of air bars **34** can be controlled by controlling the static pressure difference between the upper interior portion of the drying apparatus **10** (the portion above the coated substrate level) and the corresponding air bar plenum **35**. Independent control of the static pressure difference between the upper interior portion of the drying apparatus **10** and an air bar plenum **35** allows for independent control of the temperature and gas velocity of the top-side gas supplied by the corresponding group of air bars **34**.

Upper exhaust ports **36** are positioned above the air bars **34** to remove at least a portion of the gas supplied by the air bars **34** and can remove at least a portion of the solvent which is evaporating from the coated substrate **16**. The top-side gas exhausted by a group of upper exhaust ports **36** is exhausted into an upper exhaust plenum **37**. Five upper exhaust plenums **37** are shown, each of which is connected to two upper exhaust ports **36**. Upper exhaust ports **36** are distributed throughout the upper interior portion of the drying apparatus **10** to remove top-side gas throughout the drying apparatus **10** rather than at concentrated points. Other similar ducting arrangements are envisioned.

The gas velocity of the top-side gas through a group of upper exhaust ports **36** can largely be controlled by controlling the static pressure difference between the upper interior portion of the drying apparatus **10** and some suitable reference point (e.g., the coating room in which the coating apparatus **26** is positioned, or each upper exhaust plenum **37**). Consequently, independent control of the static pressure difference between the upper interior portion of the drying apparatus **10** and each upper exhaust plenum **37** allows for independent control of the gas velocity exhausted by the group of upper exhaust ports **36** of each upper exhaust plenum **37**.

FIG. 10 illustrates a side view of an air bar **34**. Top-side gas is shown exiting two openings. The length of the openings for the air bar **34** can be approximately equal to or less than the length of the air bar **34**. If each opening were instead a series of discrete holes rather than a single opening, the air bar **34** would be considered a perforated plate, or even a foraminous plate. A perforated or foraminous plate could be used in place of the air bar **34**, as could other sources of top-side gas (e.g., air turn, air foil).

The locations of pyrometers **38**, static pressure gages **39**, and anemometers **40** are shown in FIG. 5. These known instruments can be used to measure the temperature, static pressure, and gas velocity of the drying gas at various locations within the drying apparatus **10**. The measurements taken by these instruments can be directed to a central processing unit or other controlling mechanism (not shown) which can be used to control the conditions within the oven **10** by altering the drying gas temperature and pressure within the plenums.

To provide the necessary heat to the coated substrate to evaporate the coating solvent (i.e., the solvent portion of the coating), the drying gas can be air or an inert gas. Or, the use of a drying gas can be replaced or augmented with the use of heated rolls **50** on which the coated substrate can ride, as shown in FIG. 11. Similarly, infrared heat can be used in place of the drying gas such as with the spaced infrared heaters shown in FIG. 12 or with a heated plate positioned above or below the coated substrate **16**. The temperature of

each heated roller **50** or infrared heater **52** (or a group of rollers **50** or infrared heaters **52**) can be independently controlled.

#### Methods For Drying Using the Drying Apparatus **10**

It has been found that coatings can be dried without introducing significant mottle defects by controlling the heat transfer rate to the coating **12** and by minimizing disturbances of the gas adjacent to the coated side of the coated substrate **16** (i.e., top-side gas; see Examples Section). When the coating solvent is evaporated using a drying gas, as for example in a drying apparatus **10**, the heat transfer rate ( $h\Delta T$ ) to the coated substrate is the product of the heat transfer coefficient of the drying gas ( $h$ ) and the difference in temperature ( $\Delta T$ ), between the temperature of the drying gas in contact with it ( $T_{gas}$ ) and the temperature of the coated substrate ( $T_{cs}$ ). (The temperature of the coating **12** is assumed to be equivalent to the temperature of the coated substrate. The heat transfer rate to the coating **12** is the key to preventing or minimizing mottle formation.) In order to prevent mottle formation in the coating **12** during drying, this heat transfer rate ( $h\Delta T$ ) to the coating **12** must be kept below a threshold mottle-causing value. When a particular substrate **14** is used, the heat transfer rate to the coated substrate **16** must be kept below a corresponding threshold mottle-causing value.

As a particular coating **12** is dried (or otherwise solidified), it will eventually reach a point in which it becomes virtually mottle-proof. At this point, the heat transfer rate can be significantly increased by increasing the temperature difference  $\Delta T$  and/or by increasing the heat transfer coefficient  $h$  (e.g., by increasing the velocity of the drying gas on either the coated side or the non-coated side of the coated substrate **16**).

For a typical drying zone, the heat transfer coefficient  $h$  and the drying gas temperature  $T_{gas}$  are relatively constant and the temperature of the coated substrate **16** (and the coating **12**) increases as the coated substrate **16** is heated. Therefore, the product ( $h\Delta T$ ) has its maximum value at the initial point of the zone. Often, it is sufficient to keep the initial heat transfer rate to the coating ( $h\Delta T_i$ ) below a maximum allowable (threshold) value in order to avoid mottle in a particular drying zone.

The most efficient process for drying a coating (i.e., evaporating a coating solvent) will be one that adds heat most quickly without causing mottle. As the coated substrate temperature  $T_{cs}$  increases, the heat transfer rate ( $h\Delta T$ ) decreases along the drying zone making the drying zone less efficient (due to the smaller  $\Delta T$ ). The total amount of heat transferred to the coated substrate ( $q$ ) can be calculated by integrating the product ( $h\Delta T$ ) across the length of the oven and the width of the coating. When the coating width is relatively constant, the total amount of heat transferred to the coated substrate **16** is proportional to the area under the heat transfer rate curves described and shown below. Maximizing the area under the curve maximizes the heat transferred to the coated substrate and maximizes the efficiency of the drying process.

The maximum allowable or threshold heat transfer rate of a particular coating varies proportionately to the viscosity of the coating **12**. A coating having less thickness or a higher viscosity would have a higher maximum allowable or threshold heat transfer rate. This also means that, as the coating **12** is further dried, the viscosity will increase and the coating thickness will decrease thereby increasing the threshold heat transfer rate. Consequently, the coating can be heated at an increasingly higher heat transfer rate as the threshold temperature curve allows. Furthermore, the coat-

ing **12**, as previously noted, will eventually be dried to a point of being mottle-proof (i.e., not susceptible to mottle by the gas temperature nor by the gas velocity and any other factor affecting the heat transfer coefficient  $h$ ).

In the following discussion, the heat transfer coefficient  $h$ , of the drying gas is kept constant and the drying gas temperature  $T_{gas}$  is allowed to vary. When there is a maximum heat transfer rate ( $h\Delta T_{max}$ ) that can occur without causing mottle, there will then be a given maximum allowable difference between the temperature of the drying gas and the temperature of the coated substrate **16**.

Instead of varying the gas temperature, the temperature can be held constant while varying the heat transfer coefficient  $h$ . If the velocity of the drying gas is used to vary the heat transfer coefficient, the velocity must be kept below a maximum allowable or threshold velocity to prevent mottle.

The advantage of the additional zones is described in the Examples Section and illustrated in FIGS. 13-22. Table 1 below shows typical drying gas and coated substrate temperatures for the drying conditions described below and for a particular coated substrate **16**. Cooling of the web due to solvent evaporation is assumed negligible for the discussion below.

TABLE 1

Typical Drying Conditions Which Correspond With FIGS. 13-22

|                                        |                               |
|----------------------------------------|-------------------------------|
| Heat Transfer Coefficient - $h$        | 5 cal/sec-m <sup>2</sup> ° C. |
| Initial Coated Substrate               | 20° C.                        |
| Temperature $T_{cs}$ i                 |                               |
| Maximum Heat Transfer Rate             | 150 cal/sec-m <sup>2</sup>    |
| Without Mottle Formation - $h\Delta T$ |                               |
| Drying Length                          | 30 m                          |
| Width of Coating on Substrate          | 1 m                           |

FIG. 13 shows typical temperature curves for the coated substrate **16**. The coated substrate **16**, initially at 20° C., is subjected to a constant drying gas temperature of 50° C. The temperature of the coated substrate **16** slowly increases over the length of the drying zone (30 m) until it reaches the temperature of the drying gas. FIG. 14 shows the product  $h\Delta T$  at any given location as drying proceeds. At all times, the heat transfer rate is at or below the maximum allowable heat transfer rate of 150 cal/sec-m<sup>2</sup> and mottle is not caused. The amount of heat transferred to the coated substrate **16** per unit time drops off as the temperature of the coated substrate  $T_{cs}$  increases. At the end of the drying zone this amount is significantly less than the maximum allowable heat transfer rate. Thus, the process is much less efficient than it could be.

FIGS. 15 and 16, demonstrate the advantage when the drying process is divided into two equal zones. The advantage of the second zone is that the drying gas temperature,  $T_{gas}$  can be increased allowing the product  $h\Delta T$  to increase and drying in the second zone can take place more rapidly. Again, at all times the product  $h\Delta T$  is kept below 150 cal/sec-m<sup>2</sup>, the maximum allowable heat transfer rate without causing mottle. It should be noted that the total heat transferred to the coated substrate, represented by the area under the heat transfer rate curve in FIG. 16 is now considerably larger than for the case where only one zone is used.

Similarly, FIGS. 17 and 18 demonstrate that the total amount of heat transferred for drying is even greater and the process more efficient when three heating environments or zones are used. When 15 heating environments or zones are used as shown in FIGS. 19 and 20, the process is even more efficient. In an extreme limit, where the drying environments or zones are infinitesimally small in size and infinite in number, the drying gas temperature can be continuously

increased to maximize the allowable heat transfer rate to the coated substrate while still avoiding mottle.

FIGS. 13–20 represent a simplified case. In reality, as the coating solvent begins to evaporate (e.g., coating begins to dry), its viscosity increases and its thickness decreases. As a result, the maximum possible heat transfer rate ( $h\Delta T$ ) to the partially dried coating can be increased without formation of mottle. FIGS. 21–22 show that by increasing the heat transfer rate to correspond to the increasing maximum allowable heat transfer rate, the rate of drying can be increased even more rapidly than the simplified case shown in FIGS. 19–20 in which maximum allowable heat transfer rate is assumed constant.

Table 2 shows the total amount of heat ( $q$ ) transferred to the coated substrate for different numbers of drying environments or zones.

TABLE 2

| Drying Variables for FIGS. 13–19, and 22 |                                            |                     |
|------------------------------------------|--------------------------------------------|---------------------|
| Subzones                                 | Total Amount of Heat Transferred (cal/sec) | Corresponding FIGS. |
| 1                                        | 1427                                       | 13, 14              |
| 2                                        | 2389                                       | 15, 16              |
| 3                                        | 2936                                       | 17, 18              |
| 15                                       | 4269                                       | 19, 20              |
| $\infty$                                 | 4500                                       | No Figure           |
| 15*                                      | 5070                                       | 21, 22              |

\*With increasing maximum allowable heat transfer rate.

Further advantages and efficiency can be gained by using subzones of unequal size. For example, a larger number of smaller subzones will be advantageous in regions where the maximum allowed heat transfer rate is changing most quickly. It is also possible for evaporative cooling to lower the temperature of the coated substrate  $T_{CS}$  within a drying subzone and the product ( $h\Delta T$ ) would then be at a maximum at some intermediate point within the subzone.

As previously noted, one aspect of a method for drying includes controlling the temperature and the heat transfer coefficient  $h$  within locations or subzones of the drying oven 10, in particular, the first zone 18. This can be accomplished primarily by controlling the temperature and gas velocity of the drying gas delivered by the air foil plenums 31 and removed by the lower exhaust plenum 33. The rate at which a particular air foil plenum 31 supplies drying gas and the rate at which the corresponding lower exhaust plenum 33 removes the drying gas allows a user to balance the two and virtually create a subzone having a particular gas temperature and velocity. Similar control of corresponding pairs of plenums 31, 33 allow for control of the temperature and gas velocity of the drying gas within several subzones. As a result, the heat transfer rate to the coating 12 can be controlled and maximized within several subzones. Within a first subzone, for example, the velocity of the gas on the coated side and relative to the coated side should be not greater than a top-side gas velocity threshold, such as 150 ft/min (46 m/min) to protect a mottle-susceptible photothermographic coating 12 (e.g., the photothermographic coating described in Example 1 below).

It is important to further note that the first zone 18 is shown as an open body. In other words, the first zone 18 is shown as not including slotted vertical walls (or other physical structures with openings) to act as a barriers between the previously described subzones. Control of the heat transfer rate within individual subzones can be accomplished without the need for physical barriers. Although

physical barriers could be used, they are not needed nor preferred due to possibly adverse air flow effects which can result (i.e., high velocity flow of drying gas through the slot in a vertical wall). In addition, physical barriers with openings between the subzones (to allow transport of the moving coated substrate) could be used. But, preferably, the openings would be sufficiently large to minimize the pressure differential between subzones such that the formation of mottle is minimized or prevented.

It is also important to note that the temperature and gas velocity of the drying gas within a particular subzone and within the first zone 18 as a whole can be controlled with the use of the previously noted pyrometers 38, static pressure gauges 39, anemometers 40, and the previously noted controlling mechanism (not shown). The pyrometers 38 can sense the temperature of the coated substrate  $T_{CS}$ . The static pressure gauges 39 can sense the static pressure difference between a location within the interior of the drying apparatus 10 and some reference point (such as outside the drying apparatus 10 or within a nearby plenum). The anemometers 40 can sense the velocity of the drying gas.

The measurements from the pyrometers 38, static pressure gauges 39, and the anemometers 40 can allow the controlling mechanism and/or a user to adjust the heat transfer rate (temperature of the drying gas, heat transfer coefficient) to minimize mottle formation (at or below the maximum allowable or threshold heat transfer rate). For example, the pyrometers 38 can be positioned to sense the actual temperature of the coated substrate  $T_{CS}$  as the coated substrate is exiting one subzone and entering a downstream subzone. Based on that actual temperature versus a targeted temperature, the previously noted controlling mechanism can determine and set the heat transfer rate in the downstream subzone to be at or below the maximum allowable or threshold heat transfer rate. This controlling ability could be referred to as a feedforward strategy for a temperature set point.

Similarly, the controlling mechanism could compare the actual and the targeted temperatures and adjust the heat transfer rate in an upstream subzone to be at or below the maximum allowable or threshold heat transfer rate. This controlling ability could be referred to as a feedback loop or strategy. The targeted temperature, previously noted, can be experimentally determined so that the heat transfer rate to the coated substrate 16 can be monitored and adjusted accordingly.

Having both static pressure gauges 39 and anemometers 40, a user has the choice as to how to control the gas velocity and direction. These two instruments could be used individually or in a coordinated fashion to control gas velocity and direction by controlling the volume of gas being exhausted from the drying apparatus 10.

Control of the static pressure differences within the first zone 18 can be used to manage the gas flow through the first zone 18. While the gas within each subzone was previously described as being managed such that gas flow from subzone to another is minimized, controlling static pressure differences across the entire first zone 18 can provide the ability to create a controlled degree of gas flow from one subzone to another. For example, the pressure  $P_1$  within an upstream upper exhaust plenum 37 could be slightly higher than the pressure  $P_2$  in a downstream upper exhaust plenum 37 such that the top-side gas flows at a low velocity in the downstream direction (i.e., cocurrent flow). This could be intentionally done to create a gas velocity of the top-side gas that approximately matches the velocity of the coated substrate 16. Matching the velocities in this way can minimize dis-

turbances on the coated side of the coated substrate **16**. Alternatively, a countercurrent flow could be induced instead of the cocurrent flow; or, a combination of cocurrent and countercurrent flows could be induced.

One can control static pressure differences to manage gas flow between the upper and lower interior portions of the drying apparatus **10**. For example, setting the pressure  $P_{top}$  above the coated substrate **16** at a higher value than the pressure  $P_{bottom}$  below the coated substrate **16** biases the exhaust of the gas to the lower interior portion. This approach may be desired to prevent the hotter drying gas below the coated substrate from flowing upwardly and contacting the coating. Alternatively, the pressures could be biased oppositely so that a portion of the drying gas below the coated substrate flows upwardly and is exhausted from the upper exhaust ports **36**, or the pressures could be adjusted such that flow between the upper and lower interior portions of the drying apparatus **10** is minimized.

It is also important to note that when the temperature of the coating **12** is increased to be virtually the same as the temperature of the drying gas, the flow of the drying gas can be reduced. Similarly, when the temperature of the coating **12** is increased to a desired temperature (even if different from the drying gas temperature), again, the flow of the drying gas can be reduced. This results in more a more efficient evaporating process. In other words, less energy is required and less cost is involved.

It is also important to note that the heat transfer coefficient  $h$  has been primarily discussed as being controlled by the velocity of the drying gas. Other factors that affect the heat transfer coefficient  $h$  include the distance between the air foil **30** and the coated substrate **16**, the density of the drying gas, and the angle at which the drying gas strikes or impinges upon the coated substrate **16**. For embodiments of the present invention which includes heating means other than air foils and air bars (e.g., perforated plates, infrared lamps, heated rollers, heated plates, and/or air turns), additional factors affecting the heat transfer coefficient are present. Materials Particularly Suited For Drying By Drying Apparatus **10**

Any mottle-susceptible material, such as graphic arts materials and magnetic media, can be dried using the above-described drying apparatus **10** and methods. Materials particularly suited for drying by the drying apparatus **10** are photothermographic imaging constructions (e.g., silver halide-containing photographic articles which are developed with heat rather than with a processing liquid). Photothermographic constructions or articles are also known as "dry silver" compositions or emulsions and generally comprise a substrate or support (such as paper, plastics, metals, glass, and the like) having coated thereon: (a) a photosensitive compound that generates silver atoms when irradiated; (b) a relatively non-photosensitive, reducible silver source; (c) a reducing agent (i.e., a developer) for silver ion, for example for the silver ion in the non-photosensitive, reducible silver source; and (d) a binder.

Thermographic imaging constructions (i.e., heat-developable articles) which can be dried with the drying apparatus **10** are processed with heat, and without liquid development, are widely known in the imaging arts and rely on the use of heat to help produce an image. These articles generally comprise a substrate (such as paper, plastics, metals, glass, and the like) having coated thereon: (a) a thermally-sensitive, reducible silver source; (b) a reducing agent for the thermally-sensitive, reducible silver source (i.e., a developer); and (c) a binder.

Photothermographic, thermographic and photographic emulsions used in the present invention can be coated on a

wide variety of substrates. The substrate (also known as a web or support) **14**, can be selected from a wide range of materials depending on the imaging requirement. Substrates may be transparent, translucent or opaque. Typical substrates include polyester film (e.g., polyethylene terephthalate or polyethylene naphthalate), cellulose acetate film, cellulose ester film, polyvinyl acetal film, polyolefinic film (e.g., polyethylene or polypropylene or blends thereof), polycarbonate film and related or resinous materials, as well as aluminum, glass, paper, and the like.

## EXAMPLES

The following examples provide exemplary procedures for preparing and drying articles of the invention. Photothermographic imaging elements are shown. All materials used in the following examples are readily available from standard commercial sources, such as Aldrich Chemical Co., Milwaukee, Wis., unless otherwise specified. All percentages are by weight unless otherwise indicated. The following additional terms and materials were used.

Acryloid<sup>TM</sup> A-21 is an acrylic copolymer available from Rohm and Haas, Philadelphia, Pa.

Butvar<sup>TM</sup> B-79 is a polyvinyl butyral resin available from Monsanto Company, St. Louis, Mo.

CAB 171-15S is a cellulose acetate butyrate resin available from Eastman Kodak Co.

CBBA is 2-(4-chlorobenzoyl) benzoic acid.

1,1-bis(2-hydroxy-3,5-dimethylphenyl)-3,5,5-trimethylhexane [CAS RN=7292-14-0] is available from St-Jean Photo Chemicals, Inc., Quebec. It is a reducing agent (i.e., a hindered phenol developer) for the non-photosensitive reducible source of silver. It is also known as Nonox<sup>TM</sup> and Permanax<sup>TM</sup> WSO.

THDI is a cyclic trimer of hexamethylenediisocyanate. It is available from Bayer Corporation Co., Pittsburgh, Pa. It is also known as Desmodur<sup>TM</sup> N-3300.

Sensitizing Dye-1 is described in U.S. Pat. No. 5,393,654 which is hereby incorporated by reference. It has the structure shown below.



2-(Tribromomethylsulfonyl)quinoline is disclosed in U.S. Pat. No. 5,460,938 which is hereby incorporated by reference. It has the structure shown below.



The preparation of Fluorinated Terpolymer A (FT-A) is described in U.S. Pat. No. 5,380,644, which is hereby incorporated by reference. It has the following random polymer structure, where m=70, n=20 and p=10 (by weight % of monomer).



## Example 1

A dispersion of silver behenate pre-formed core/shell soap was prepared as described in U.S. Pat. No. 5,382,504 which is hereby incorporated by reference. Silver behenate, Butvar™ B-79 polyvinyl butyral and 2-butanone were combined in the ratios shown below in Table 3.

TABLE 3

| Silver behenate dispersion |                |
|----------------------------|----------------|
| Component                  | Weight Percent |
| Silver behenate            | 20.8%          |
| Butvar™ B-79               | 2.2%           |
| 2-Butanone                 | 77.0%          |

Then, a photothermographic emulsion was prepared by adding 9.42 lb. (4.27 Kg) of 2-butanone and a premix of 31.30 g of pyridinium hydrobromide perbromide dissolved in 177.38 g of methanol to 95.18 lb. (43.17 Kg) of the pre-formed silver soap dispersion. After 60 minutes of mixing, 318.49 g of a 15.0 wt % premix of calcium bromide in methanol was added and mixed for 30 minutes. Then, a premix of 29.66 g of 2-mercapto-5-methylbenzimidazole, 329.31 g of 2-(4-chlorobenzoyl)benzoic acid, 6.12 g of Sensitizing Dye-1, and 4.76 lb. (2.16 Kg) of methanol was added. After mixing for 60 minutes, 22.63 lb. (10.26 Kg) of Butvar™ B-79 polyvinyl butyral resin was added and allowed to mix for 30 minutes. After the resin had dissolved, a premix of 255.08 g of 2-(tribromomethylsulfonyl) quinoline in 6.47 lb. (2.93 Kg) of 2-butanone was added and allowed to mix for 15 minutes. Then 5.41 lb. (2.45 Kg) of 1,1-bis(2-hydroxy-3,5-dimethylphenyl)-3,5,5-trimethylhexane was added and mixed for another 15 minutes. Then a premix of 144.85 g of THDI and 72.46 g of 2-butanone was added and mixed for 15 minutes. Next, 311.61 g of a 26.0% solution of tetrachlorophthalic acid in 2-butanone was added and mixed for 15 minutes. Finally, a solution of 243.03 g of phthalazine and 861.64 g of 2-butanone was added and mixed for 15 minutes.

A top-coat solution was prepared by adding 564.59 g of phthalic acid to 30.00 lb. (13.61 Kg) of methanol and mixing until the solids dissolved. After adding 174.88 lb. (79.3 Kg) of 2-butanone, 149.69 g of tetrachlorophthalic acid was added and mixed for 15 minutes. Then, 34.38 lb. (15.59 Kg) of CAB 171-15S resin was added and mixed for 1 hour. After the resin had dissolved, 2.50 lb. (1.13 Kg) of a 15.0 wt-% solution of FT-A in 2-butanone was added and mixed for 10 minutes. Then a premix of 26.33 lb. (11.94 Kg) of

2-butanone and 630.72 g of Acryloid A-21 resin and a premix of 26.33 lb. (11.94 Kg) of 2-butanone, 796.60 g of CAB 171-15S resin, and 398.44 g of calcium carbonate were added and mixed for 10 minutes.

A drying apparatus 10A like that shown in FIG. 23 herein was used to prepare a photothermographic article. (The first zone 18A within the drying apparatus 10A shown in FIG. 23 does not have the ability to create subzones.) A polyester substrate having a thickness of 6.8 mil (173  $\mu$ m) was simultaneously coated with the photothermographic emulsion and top-coat solutions at 75 ft/min (0.38 meters per second). The photothermographic emulsion layer was applied at a wet thickness of 3.2 mil (81.3  $\mu$ m). The top-coat solution was applied at a wet thickness of 0.75 mil (19.1  $\mu$ m). After passing the coating die, the coated substrate 16A traveled a distance of about 13 feet (4 meters) and passed through an entrance slot into a dryer composed of 3 zones. The first zone 18A was comprised of air foils 30A below the coated substrate 16A which provided drying gas and also provide flotation for the coated substrate 16A. There were also perforated plate-type air bars 34A positioned 20 centimeters above the coated substrate 16A which provided top-side gas to maintain safe operating conditions below the lower flammability limit of the solvent. The majority of the drying heat is provided by the backside airfoils 30A (i.e., 10) heat provided from below the substrate 14A to the coating 12A). The air temperature was set to the same value in each zone, however, the air pressure, hence the air velocity, was independently controlled for the air foils 30A and air bars 34A. The coating 12A was dried to be mottle proof within the first oven zone. The second and third oven zones 20A, 21A used counter-current parallel air flow and served to remove the residual solvent. (In the figures, air flow direction is shown with the included arrows.)

The variables investigated were the temperature of the drying gas  $T_{gas}$  and heat transfer coefficient  $h$ . The heat transfer coefficient  $h$  was varied by adjusting the air foil pressure drop and was measured independently.

The presence and severity of mottle was determined by preparing "greyouts." Greyouts are samples that have been uniformly exposed to light and developed at 255° F. (124° C.) using a heated roll processor (not shown) so that they have a uniform Optical Density, for example between 1.0 and 2.0.

The amount of mottle was subjectively determined by comparing samples placed on a light box. The developed films were visually inspected for mottle and rated relative to one another. Mottle was rated as high, medium, or low.

The conditions used in the first zone 18A and results obtained are summarized below in Table 4. As  $\Delta P_{bot}$  or  $T_{gas}$  was increased, the level of mottle was increased.

TABLE 4

| Example | First Zone Conditions     |                           |                     |                             |               |
|---------|---------------------------|---------------------------|---------------------|-----------------------------|---------------|
|         | $\Delta P_{bot}$<br>(kPa) | $\Delta P_{top}$<br>(kPa) | $T_{gas}$<br>(° C.) | $\Delta P_{static}$<br>(Pa) | Mottle Rating |
| 1-1     | 0.125                     | 0.025                     | 37.8                | -0.5                        | Low           |
| 1-2     | 0.500                     | 0.025                     | 37.8                | -0.5                        | Medium        |
| 1-3     | 0.125                     | 0.025                     | 60.0                | -0.5                        | High          |

$\Delta P_{bot}$  is the pressure drop across the airfoils 31A.

$\Delta P_{top}$  is the pressure drop across the air bars 34A.

$T_{gas}$  is the temperature of the heated drying gas.

$\Delta P_{static}$  is the pressure drop between the first zone 18A and the coater room (not shown).

Drying more harshly increased the severity of the mottle. If one were to consider increasing the drying conditions only

in terms of the available operating parameters, one would not make the appropriate conclusions concerning the affects on mottle. Changing the pressure drop from 0.125 to 0.5 kPa is a factor of 4 increase. An appropriate temperature measure is the difference between the drying gas and the substrate as it enters the zone. This temperature measure increases a factor of 2.3 as the gas temperature increased from 37.8 to 60° C. One would expect that changing the air foil pressure drop would have the larger effect on mottle, however, the opposite is true.

In order to determine the effect on mottle, one needs to consider a more appropriate measure such as the product of the heat transfer coefficient and the difference between the temperature of the drying gas  $T_{gas}$  and the temperature of the coated substrate  $T_{cs(i)}$  as it enters the zone. This product is the rate of heat transferred to the film and is a direct measure of the rate of heating of the film. As shown below in Table 5, increasing the initial rate of heat transfer to the film, ( $h\Delta T_i$ ), increased the severity of mottle.

TABLE 5

| Example | $\Delta P_{bar}$<br>(kPa) | $T_{gas}$<br>(° C.) | $T_{cs(i)}$<br>(° C.) | $h$<br>(cal/m <sup>2</sup> s K) | $h\Delta T_i$<br>(cal/m <sup>2</sup> s) | Mottle Rating |
|---------|---------------------------|---------------------|-----------------------|---------------------------------|-----------------------------------------|---------------|
| 1-1     | 0.125                     | 37.8                | 21.1                  | 13.7                            | 229                                     | Low           |
| 1-2     | 0.500                     | 37.8                | 21.1                  | 19.4                            | 324                                     | Medium        |
| 1-3     | 0.125                     | 60.0                | 21.1                  | 13.7                            | 532                                     | High          |

The term  $\Delta T_i$  indicates the difference between  $T_{gas}$  and  $T_{cs(i)}$ . The term  $T_{cs(i)}$  is the initial temperature of the coated substrate just before it enters the drying apparatus 10A.

### Example 2

Using the coating materials and oven described in Example 1, the photothermographic emulsion and top-coat solution were simultaneously coated at 3.6 mil (91.4  $\mu$ m) and 0.67 mil (17.0  $\mu$ m) respectively on 6.8 mil (173  $\mu$ m) polyester substrate. Greyouts were prepared and rated as described in Example 1. The drying conditions used and results obtained, which are shown below in Table 6, demonstrate that as the initial heat transfer rate to the film ( $h\Delta T_i$ ) was increased, the severity of mottle increased. More specifically, at a constant heat transfer coefficient, as the initial temperature difference between the coating 12A and the drying gas was increased, the severity of mottle increased.

TABLE 6

| Example | $T_{gas}$<br>(° C.) | $T_{cs(i)}$<br>(° C.) | $h$<br>(cal/m <sup>2</sup> s K) | $h\Delta T_i$<br>(cal/m <sup>2</sup> s) | Mottle Rating |
|---------|---------------------|-----------------------|---------------------------------|-----------------------------------------|---------------|
| 2-1     | 37.8                | 21.1                  | 13.7                            | 229                                     | Low           |
| 2-2     | 51.7                | 21.1                  | 13.7                            | 419                                     | Medium        |
| 2-3     | 82.2                | 21.1                  | 13.7                            | 837                                     | High          |

### Example 3

Solutions were prepared as described in Example 1 and were simultaneously coated on a polyester substrate at 100 ft/min (0.508 meters per second). After passing the coating die, the substrate traveled a distance of approximately 10 feet (3 meters) and then passed through a slot into a dryer with 3 zones similar to FIG. 3. The gas velocity of the counter-current parallel flow air was held constant and the temperature was varied as shown below in Table 7. As the initial rate of heat transfer ( $h\Delta T_i$ ) to the coated substrate 16 was increased, the severity of mottle increased. Without

considering the value of the heat transfer coefficient  $h$ , no direct comparisons between the ovens in Examples 2 and 3 is possible.

TABLE 7

| Example | $T_{gas}$<br>(° C.) | $T_{cs(i)}$<br>(° C.) | $h$<br>(cal/m <sup>2</sup> s K) | $h\Delta T_i$<br>(cal/m <sup>2</sup> s) | Mottle Rating |
|---------|---------------------|-----------------------|---------------------------------|-----------------------------------------|---------------|
| 3-1     | 93.3                | 21.1                  | 2.85                            | 206                                     | Low           |
| 3-2     | 71.1                | 21.1                  | 2.58                            | 129                                     | Very Low      |

### Example 4

Solutions were prepared as described in Example 1 and were simultaneously coated on a polyester substrate at 25 ft/min (0.127 meters per second). After passing the coating die, the substrate traveled a distance of 10 ft (3 meters) and then passed through a slot into a dryer with 3 zones similar to the first zone 18A of FIG. 23. This is an oven with air foils on the bottom, air bars on the top, and an overall flow of air through the oven. The atmosphere is inert gas and the partial pressure of solvent could be controlled using a condenser loop. The experimental conditions are shown below in Tables 8 (Zone 1) and 9 (Zone 2). As the product ( $h\Delta T_i$ ) was increased in the Zone 1, the severity of mottle was increased. Also, for a given product ( $h\Delta T_i$ ) in Zone 1, the product ( $h\Delta T_i$ ) in Zone 2 affected mottle. When the coating was not yet mottle-proof and was entering Zone 2, decreasing the product ( $h\Delta T_i$ ) in Zone 2 caused a reduction in the severity of mottle.

TABLE 8

| Zone 1  |                     |                       |                                 |                                         |
|---------|---------------------|-----------------------|---------------------------------|-----------------------------------------|
| Example | $T_{gas}$<br>(° C.) | $T_{cs(i)}$<br>(° C.) | $h$<br>(cal/m <sup>2</sup> s K) | $h\Delta T_i$<br>(cal/m <sup>2</sup> s) |
| 4-1     | 82.2                | 21.1                  | 29.0                            | 1770                                    |
| 4-2     | 37.8                | 21.1                  | 18.9                            | 316                                     |
| 4-3     | 37.8                | 21.1                  | 18.9                            | 316                                     |

TABLE 9

| Zone 2  |                     |                       |                                 |                                         |
|---------|---------------------|-----------------------|---------------------------------|-----------------------------------------|
| Example | $T_{gas}$<br>(° C.) | $T_{cs(i)}$<br>(° C.) | $h$<br>(cal/m <sup>2</sup> s K) | $h\Delta T_i$<br>(cal/m <sup>2</sup> s) |
| 4-1     | 82.2                | 71.1                  | 29.7                            | 329                                     |
| 4-2     | 60                  | 26.7                  | 24.0                            | 799                                     |
| 4-3     | 60                  | 37.8                  | 24.2                            | 537                                     |

Reasonable modifications and variations are possible from the foregoing disclosure without departing from either the spirit or scope of the present invention as defined by the claims.

We claim:

1. A method for evaporating a coating solvent from a coating on a substrate and for reducing the formation of drying mottle as the coating solvent is evaporating, the substrate having a first substrate surface and a second substrate surface, the method comprising the steps of:
  - (a) applying the coating onto the first substrate surface, the coating having a first coating temperature;
  - (b) heating the coating with a first drying gas at no faster than a first heat transfer rate, the first drying gas having a first drying gas temperature, the first heat transfer rate

being created by a first heat transfer coefficient and a first temperature difference between the first coating temperature and the first drying gas temperature, the first heat transfer rate causing maximum evaporation of the coating solvent yet no more than an acceptable level of drying mottle, the coating being heated predominantly by heat transferred from the first drying gas and through the substrate second surface; and

(c) heating the coating with a second drying gas at no faster than a second heat transfer rate greater than the first heat transfer rate after a first portion of the coating solvent has evaporated, the coating having a second coating temperature just before being heated by the second drying gas, the second drying gas having a second drying gas temperature, the second heat transfer rate being created by a second heat transfer coefficient and a second temperature difference between the second coating temperature and the second drying gas temperature, the second heat transfer rate causing a maximum evaporation of the coating solvent yet no more than an acceptable level of drying mottle, at least one of the second heat transfer coefficient and the second temperature difference being greater than the respective first heat transfer coefficient and first temperature difference, the coating being heated predominantly by heat transferred from the drying gas and through the substrate second surface.

2. The method of claim 1, further comprising the step of heating the coating with a third drying gas at no higher than a third heat transfer rate after a second portion of the coating solvent has evaporated and the coating has a third wet thickness and a third viscosity, the coating having a third coating temperature just before being heated by the third drying gas, the third wet thickness being less than the second wet thickness, the third drying gas having a third drying gas temperature, the third heat transfer rate being created by a third heat transfer coefficient and a third temperature difference between the third coating temperature and the third drying gas temperature, the third heat transfer rate causing maximum evaporation of the coating solvent and no more than an acceptable level of mottle when the coating is at the third wet thickness and the third viscosity, at least one of the third heat transfer coefficient and the third drying gas temperature being greater than the respective second heat transfer coefficient and second drying gas temperature, the coating being heated predominantly by the drying gas adjacent to the substrate second surface.

3. The method of claim 2, the second viscosity being greater than the first viscosity, the third viscosity being greater than the second viscosity.

4. The method of claim 2, the second heat transfer rate being greater than the first heat transfer rate, the third heat transfer rate being greater than the second heat transfer rate.

5. The method of claim 2, the step of heating the coating at no higher than the third heat transfer rate comprising heating the coating approximately at the third heat transfer rate.

6. The method of claim 2, further comprising the step of determining at least one of when the coating has reached the third coating temperature and when the second portion of the coating solvent has evaporated.

7. The method of claim 1, the step of heating the coating at no higher than the first heat transfer rate comprising heating the coating approximately at the first heat transfer rate, and the step of heating the coating at no higher than the second heat transfer rate comprising heating the coating approximately at the second heat transfer rate.

8. The method of claim 1, further comprising the step of determining at least one of when the coating has reached the second coating temperature and when the first portion of the coating solvent has evaporated.

9. The method of claim 1, a third gas being present adjacent the substrate first surface, the third gas having a third gas velocity relative to the substrate first surface, the method further comprising the step of maintaining the third gas velocity to not greater than a third gas velocity threshold to produce no more than an acceptable level of mottle in the coating.

10. The method of claim 9, the third gas velocity threshold being 46 meters per minute.

11. The method of claim 1, the substrate traveling in a substrate travel direction, the drying gas adjacent to the substrate second surface being at least one of drying gas impinging on the substrate second surface, drying gas flowing generally cocurrently with the substrate travel direction, drying gas flowing generally countercurrently to the substrate travel direction, drying gas flowing generally orthogonally to the substrate travel direction, and the drying gas flowing generally diagonally to the substrate travel direction.

12. The method of claim 1, wherein the coating is useful in making one of an imaging medium and a data storage medium.

13. A method for evaporating a coating solvent from a coating on a first substrate surface and minimizing the formation of mottle in the coating as the coating solvent is evaporating, the coating having a first coating temperature  $T_{c1}$  when applied to the substrate, the substrate also having a second substrate surface opposite to the first substrate surface, the method comprising the steps of:

(a) providing a first evaporating environment for the coating, the first evaporating environment containing a first drying gas which heats the coating predominantly by flowing adjacent the second substrate surface;

(b) flowing the first drying gas adjacent the second substrate surface at a first drying gas velocity resulting in a first heat transfer coefficient  $h_1$  and heating the first drying gas to a first drying gas temperature  $T_{gas1}$  such that the product

$$h_1 (T_{gas1} - T_{c1})$$

is not greater than a first threshold value such that the formation of mottle is substantially prevented;

(c) determining the first threshold value for the product  $h_1 (T_{gas1} - T_{c1})$ ; and

(d) transporting the substrate through the first evaporating environment.

14. The method of claim 13, further comprising the steps of:

(e) providing a second evaporating environment for the coating when at a second coating temperature  $T_{c2}$ , the second evaporating environment containing a second drying gas which heats the coating predominantly by heat transferred from the second drying gas and through the second substrate;

(f) flowing the second drying gas adjacent the second substrate surface at a second drying gas velocity to create a second heat transfer coefficient  $h_2$  and heating the second drying gas to a second drying gas temperature  $T_{gas2}$  such that the product

$$h_2 (T_{gas2} - T_{c2})$$

is not greater than a second threshold value such that the formation of mottle is substantially prevented when the coating is within the second evaporating environment;

## 25

- (g) determining the second threshold value for the product  $h_2(T_{gas2}-T_{c2})$ ; and
- (h) transporting the substrate through the second evaporating environment.

15. The method of claim 14, the second heat transfer coefficient  $h_2$  being greater than the first heat transfer coefficient  $h_1$ .

16. The method of claim 14, the second drying gas temperature  $T_{gas2}$  being higher than the first drying gas temperature  $T_{gas1}$ .

17. The method of claim 14, the product

$$h_1(T_{gas1}-T_{c1})$$

being approximately at the first threshold value, and the product

$$h_2(T_{gas2}-T_{c2})$$

being approximately at the second threshold value.

18. The method of claim 14, the coating having a first mass, first thickness, first viscosity, first coating temperature, and a first percent solids before step (b) and a second mass, second thickness, second viscosity, second coating temperature, and a second percent solids after step (b), the method further comprising the steps of:

- (i) determining at least one of the second mass, second thickness, second viscosity, second coating temperature, and second percent solids; and
- (j) adjusting at least one of the second drying gas temperature  $T_{gas2}$  and the second heat transfer coefficient  $h_2$  based on the results of step (i) such that the product  $h_2(T_{gas2}-T_{c2})$

is not greater than a second threshold value.

19. The method of claim 13, a third gas being present adjacent the substrate first surface, the third gas having a third gas velocity relative to the substrate surface, the method further comprising the step of maintaining the third gas velocity to not greater than a third gas velocity threshold which substantially prevents formation of mottle in the coating.

20. The method of claim 19, the third gas velocity threshold being 46 meters per minute.

21. The method of claim 13, the substrate traveling in a substrate travel direction, the first drying gas adjacent the substrate second surface being at least one of drying gas impinging on the substrate second surface, the first drying gas flowing generally cocurrently with the substrate travel direction, the first drying gas flowing generally countercurrently to the substrate travel direction, the first drying gas flowing generally orthogonally to the substrate travel direction, and the first drying gas flowing generally diagonally to the substrate travel direction.

22. The method of claim 13, the coating having a first mass, first thickness, first viscosity, first coating temperature, and a first percent solids before step (b) and a second mass, second thickness, second viscosity, second coating temperature, and a second percent solids after step (b), the method further comprising the steps of:

- (i) determining at least one of the second mass, second thickness, second viscosity, second coating temperature, and second percent solids; and
- (j) adjusting at least one of the first drying gas temperature  $T_{gas1}$  and the first heat transfer coefficient  $h_1$  based on the results of step (i).

23. A method for evaporating a coating solvent from a coating on a substrate and minimizing the formation of drying mottle as the coating solvent is evaporating, the substrate having a first substrate surface and a second substrate surface, the method comprising the steps of:

## 26

(a) applying the coating onto the first substrate surface, the coating having a first coating temperature;

(b) heating the coating with a first drying gas having a first drying gas temperature, a first heat transfer rate being created by a first heat transfer coefficient and a first temperature difference between the first coating temperature and the first drying gas temperature, the first heat transfer rate causing a maximum evaporation of the coating solvent yet no more than an acceptable level of drying mottle, the coating being heated predominantly by heat transferred from the first drying gas and through the substrate second surface; and

(c) heating the coating with a second drying gas after a first portion of the coating solvent has evaporated, the coating having a second coating temperature just before being heated by the second drying gas, the second drying gas having a second drying gas temperature, a second heat transfer rate being created by a second heat transfer coefficient and a second temperature difference between the second coating temperature and the second drying gas temperature, the second heat transfer rate causing a maximum evaporation yet no more than an acceptable level of drying mottle, at least one of the second heat transfer coefficient and the second temperature difference being greater than the respective first heat transfer coefficient and first temperature difference such that the second heat transfer rate is greater than the first heat transfer rate, the coating being heated predominantly by heat transferred from the drying gas and through the substrate second surface.

24. The method of claim 23, further comprising the step of determining at least one of when the coating has reached the second coating temperature and when the first portion of the coating solvent has evaporated.

25. The method of claim 23, the substrate traveling in a substrate travel direction, the drying gas adjacent the substrate second surface being at least one of drying gas impinging on the substrate second surface, drying gas flowing generally cocurrently with the substrate travel direction, drying gas flowing generally countercurrently to the substrate travel direction, drying gas flowing generally orthogonally to the substrate travel direction, and the drying gas flowing generally diagonally to the substrate travel direction.

26. The method of claim 23, further comprising the step of heating the coating with a third drying gas at no higher than a third heat transfer rate after a second portion of the coating solvent has evaporated, the coating having a third coating temperature just before being heated by the third drying gas, the third drying gas having a third drying gas temperature, the third heat transfer rate being created by a third heat transfer coefficient and a third temperature difference between the third coating temperature and the third drying gas temperature, the third heat transfer rate causing maximum evaporation of the coating solvent and no more than an acceptable of mottle, at least one of the third heat transfer coefficient and the third drying gas temperature being greater than the respective second heat transfer coefficient and second drying gas temperature, the coating being heated predominantly by the drying gas adjacent the substrate second surface.

27. The method of claim 26, the second heat transfer rate being greater than the first heat transfer rate, the third heat transfer rate being greater than the second heat transfer rate.

28. The method of claim 26, the step of heating the coating at no higher than the third heat transfer rate comprising heating the coating approximately at the third heat transfer rate.

**29.** The method of claim **26**, further comprising the step of determining at least one of when the coating has reached the third coating temperature and when the second portion of the coating solvent has evaporated.

**30.** The method of claim **23**, a third gas being present adjacent the substrate first surface, the third gas having a third gas velocity relative to the substrate first surface, the method further comprising the step of maintaining the third gas velocity to not greater than a third gas velocity threshold to substantially prevent the formation of mottle in the coating.

**31.** The method of claim **30**, the third gas velocity threshold being 46 meters per minute.

**32.** A method for drying a coating on a substrate, the method comprising:

applying a first drying gas to dry the coating at no more than a first heat transfer rate, the first heat transfer rate being a function of a first heat transfer coefficient and a first temperature difference between the first drying gas and the coating;

adjusting at least one of the first heat transfer coefficient and the first temperature difference to generate a maximum rate of evaporation with no more than an acceptable level of drying mottle;

applying a second drying gas to dry the coating at no more than a second heat transfer rate after the first drying gas has partially dried the coating, the second heat transfer rate being a function of a second heat transfer coefficient and a second temperature difference between the second drying gas and the coating; and

adjusting at least one of the second heat transfer coefficient and the second temperature difference to generate a maximum rate of evaporation with no more than an acceptable level of drying mottle,

wherein at least one of the second heat transfer coefficient and the second temperature difference is greater than the first heat transfer coefficient and the first temperature difference, respectively, such that the second heat transfer rate is greater than the first heat transfer rate.

**33.** The method of claim **32**, further comprising:

applying a third drying gas to dry the coating at no more than a third heat transfer rate after the second drying gas has partially dried the coating, the third heat transfer rate being a function of a third heat transfer coefficient and a third temperature difference between the third drying gas and the coating; and

adjusting at least one of the third heat transfer coefficient and the third temperature difference to generate a maximum rate of evaporation with no more than an acceptable level of mottle,

wherein at least one of the third heat transfer coefficient and the third temperature difference is greater than the second heat transfer coefficient and second temperature difference, respectively.

**34.** The method of claim **33**, wherein the coating has a viscosity that increases as the coating is dried by the first, second, and third drying gasses.

**35.** The method of claim **33**, wherein the second heat transfer rate is greater than the first heat transfer rate, and the third heat transfer rate is greater than the second heat transfer rate.

**36.** The method of claim **32**, wherein the second temperature difference is greater than the first temperature difference.

**37.** The method of claim **32**, wherein the second heat transfer coefficient is greater than the first heat transfer coefficient.

**38.** A method for drying a coating on a substrate, the method comprising:

heating the coating with a first drying gas at a first heat transfer rate; and

heating the coating with a second drying gas at a second heat transfer rate after the coating has been partially dried to a higher viscous state by the first drying gas, wherein:

each of the first and second heat transfer rates is determined by a heat transfer coefficient of the respective gas and a temperature difference between the respective gas and the coating,

the second heat transfer rate is greater than the first heat transfer rate, and

each of the first and second heat transfer rates is selected according to the changing viscosity of the coating to produce maximum evaporation of solvent in the coating while producing no more than an acceptable level of drying mottle.

**39.** A method for drying a coating on a substrate, the method comprising:

heating the coating with a series of drying gasses at progressively higher heat transfer rates, each of the heat transfer rates being determined by a heat transfer coefficient of the respective gas and a temperature difference between the respective gas and the coating; and

selecting each of the heat transfer rates according to the changing viscosity of the coating to thereby produce maximum evaporation of solvent in the coating while producing no more than an acceptable level of drying mottle given the viscous state of the coating.

**40.** A method for drying a coating on a substrate, the method comprising:

applying a drying gas to the coating;

increasing a heat transfer rate of the drying gas as the coating becomes more viscous; and

controlling the heat transfer rate based on the viscosity of the coating to prevent formation of an unacceptable level of drying mottle.